

# UNITED STATES PATENT OFFICE.

EZECHIEL WEINTRAUB, OF NEW YORK, N. Y., ASSIGNOR TO GENERAL ELECTRIC COMPANY, A CORPORATION OF NEW YORK.

## PROCESS OF PREPARING CATALYZING MATERIAL.

1,423,978.

Specification of Letters Patent. Patented July 25, 1922.

No Drawing.

Application filed March 26, 1918. Serial No. 224,897.

To all whom it may concern:

Be it known that I, EZECHIEL WEINTRAUB, a citizen of the United States, residing at the city of New York, in the county of New York, State of New York, have invented certain new and useful Improvements in Processes of Preparing Catalyzing Material, of which the following is a specification.

The present invention comprises a process of preparing a novel form of catalyzing material, described by me in a copending application, Serial No. 224,895, filed March 26, 1918, comprising a catalyzing agent and a support therefor of fibrox, an artificial chemically inert material consisting of a mass of very fine interlacing fibres of a silicon compound. Fibrox is fully described by me in the Transactions of the American Electrochemical Society, Vol. XXVII, p. 267 (1915).

Oxidizing gases like oxygen will at elevated temperatures transform the silicon oxycarbide of which the fibres consist, into silica but as this transformation is not accompanied by change of structure, the effectiveness of the material as a catalytic support is not impaired when thus oxidized. Such transformation products of the described material which have the essential physical structure of fibrox are also to be included under the same generic name of "fibrox."

In accordance with my invention the mass of fibrox to be provided with a catalyzing material is subjected to a fluid menstruum capable of depositing the desired catalyzing agent upon the fibres throughout the mass of the fibrox.

In accordance with the preferred method of carrying out my invention fibrox is placed in a container which is exhausted and then gas, or a mixture of gases, capable of liberating the desired catalyzer is admitted. As these gases immediately permeate the fibrous mass conditions are particularly favorable for a deposition of the catalyzer upon the surface of the fibres when the mass is heated or otherwise treated to produce the desired reaction. For example, finely divided nickel may be deposited by the decomposition of nickel carbonyl vapor in contact with fibrox; platinum may be deposited on the fibrox by the reduction of carbonyl platinochloride and osmium deposition may be carried out

by the reduction of vapors of osmium tetrachloride with hydrogen.

Fibrox strips may be placed in a container of glass, quartz or the like. The air may be preferably withdrawn with a vacuum pump and the vapor of nickel carbonyl then is admitted preferably at reduced pressure, say, at about one-fifth atmosphere in order to allow for the increase in volume and pressure when the carbonyl decomposes. The container when thus charged is heated to about 180° C. in order to decompose the nickel carbonyl, depositing finely divided nickel on the fibrox fibres. This treatment may be repeated several times to produce a desired deposit.

When a deposit of platinum is desired, the fibrox is placed in a container of glass, quartz or other material sufficiently refractory and a quantity of carbonyl platinochloride is admitted, the process being the same as above described in connection with the deposition of nickel. This material may be formed in a chamber immediately adjacent the fibrox container by the action of carbon monoxide and chlorine gas on platinum sponge at a temperature of about 250° C.

In accordance with a modification of my invention, the deposition of the catalyzer may be carried out by the use of a liquid instead of a gaseous menstruum or carrier. In this case care must be exercised in the subsequent washing of the fibrox so as not to leave any salts upon the fibres as this would cause the fibrox to shrink when drying into a hard brittle mass. When it is desired to deposit a coating of nickel upon the fibrox fibres by the solution process, nickel sulphate is dissolved in water and to the solution about twice the amount of sodium hypophosphite is added which is theoretically required to reduce the nickel sulphate. The fibrox is immersed in this solution and the solution is heated to boiling.

The resulting chemical action involves the formation of nickel hypophosphite and its subsequent reduction on continuous boiling by the excess of sodium hypophosphite to form metallic nickel. The boiling is continued for at least an hour and thereupon the fibrox is removed, carefully washed with distilled water, and finally dried. If the washing operation with distilled water has

been thoroughly done so as to leave no salts upon the fibrox, then the coated fibrox will return to its initial bulk upon drying.

Similarly a mass of fibrox may be placed 5 in a solution of chlorplatinic acid and an excess of saturated solution of ferrous sulphate is added and the solution mixture is boiled. The result is a deposition of platinum on the fibres of the fibrox which 10 thereupon should be thoroughly washed with distilled water.

The fibrox catalyst may be used for the oxidation of ammonia to nitric acid, the oxidation of sulphur dioxide to form sulphur 15 trioxide for the manufacture of sulphuric acid, and particularly for the synthesis of ammonia from nitrogen and hydrogen. In this case as high pressure is used a small sized apparatus is desirable and therefore 20 the large active surface offered by fibrox for a small volume is of special advantage.

What I claim as new and desire to secure by Letters Patent of the United States, is:—

1. The method of depositing a catalyzing

material on the fibres of fibrox which consists in permeating said fibrox with a gaseous menstruum capable of liberating the desired material and then producing the desired reaction by heating the gaseous menstruum to the reaction temperature. 25

2. The method of depositing a catalyzing material on the fibres of fibrox which consists in placing a mass of fibrox to be acted upon within a container, exhausting said container, admitting a gas, or mixture of 30 gases, capable of liberating the desired material upon heating to a certain temperature and then heating said container and contents to said temperature.

3. The method of depositing nickel upon 40 a fibrous support which consists in permeating said support with nickel carbonyl in the gaseous state under pressure less than atmospheric and then heating said carbonyl to the decomposition temperature.

In witness whereof, I have hereunto set my hand this 20th day of March, 1918.

EZECHIEL WEINTRAUB.